

Nov. 24, 1931.

E. KRAMER

1,832,868

METHOD OF MANUFACTURING FOIL SHAPED METAL GRAINS

Filed Oct. 21, 1929



Inventor:  
Erwin Kramer,  
By Apprentice  
Atg.

## UNITED STATES PATENT OFFICE

ERWIN KRAMER, OF BERLIN, GERMANY, ASSIGNOR TO HARTSTOFF-METALL  
AKTIENGESELLSCHAFT, OF BERLIN, GERMANY

## METHOD OF MANUFACTURING FOIL-SHAPED METAL GRAINS

Application filed October 21, 1929, Serial No. 401,299, and in Germany October 22, 1928.

My invention relates to the manufacture of metal powders from small metal particles, the individual particles of the powder being foil-shaped and commercially known as "bronze colors". The present method constitutes an improvement of the method described in my application Serial Number 661,331. The improvement consists in rendering it possible to carry out the method in a continuous manner, in such a way, that a particularly uniform product is attained which is important for the quality of the product. At the same time, the output is increased, that is to say, not only the efficiency of the method is increased, but also the output in a certain unit of time. Another advantage of the present improved method is that the apparatus in which it is carried out need not be opened while the service is going on so that no air can find access to the bronze: when the bronze is hot it is easily affected by air, and, therefore, at all events air should be excluded. It is particularly advisable to fill the apparatus with an indifferent gas to thereby prevent disastrous explosions which are likely to occur, for instance, with aluminium bronze. Another advantage attained by the method according to this invention is this that still finer foils can be produced and at the same time these foils can be prevented from oxidizing or even burning after having left the machine as is frequently the case with aluminium bronze.

For practicing my improved method I make use of a machine in which the spreading of the metal powder particles and the flattening and smoothing of the same is effected with the aid of a current of air or other gas, preferably an indifferent gas, which is blown continually through the machine with a certain suitable strength or force, the current entering the machine on the same side where the metal powder to be treated is introduced, and leaving it at the opposite end, the strength or force of the current being such that it will carry away the finished particles from the flattening and smoothing device of the machine into a separating device in which the particles are subdivided and collected,

as will be found more fully described hereinafter.

A flattening device designed according to this invention is a longitudinally extending apparatus, preferably in the shape of a drum. 55 Since, while the flattening operation is going on, the individual particles of the metal powder are continually whirled up, and since the thinner foils have a greater floating capacity than the thicker ones, the current of air, or other gas, passing through the apparatus assists the thinner foils to pass through the apparatus from one end to the other end, and carries those which are thin enough out of the apparatus, or out of the drum respectively. 60 The thinner foils therefore, do not stay or remain as long in the drum as do the other ones which have not been so intensively acted on by the flattening members or tools. Therefore, at the charging end of the drum 70 where the unflattened particles are introduced, practically no flattened particles or only a few are present, whereas this is the case more and more in the direction toward the other end of the drum. 75

Obviously by this method an extraordinarily uniform and also economically good spreading of the particles is attained. This effect is further promoted by the circumstance that the finished particles leave the drum quickly and on the shortest way, and do not, therefore, remain longer in the drum than absolutely necessary. If the particles would remain in the drum longer than is requisite they would be acted on more than is favorable whereby the drum would be too much clogged and the consumption of power would be increased. Also the working of the particles by the flattening members would be impeded. 85

Another advantage resulting from the present improved method is that difficulties hitherto encountered are overcome. It can occur that particles which have already been 95 acted on to a certain degree contact with one another and remain in contact so as to form a body of a certain bulk upon which the current of air or other gas passing through the drum cannot act in the desired manner.

As the foils float slowly in the drum the 100

flattening members or tools, viz. steel balls, can knock them effectively to the bottom of the drum and beat and flatten them there.

5 A long drum for carrying through the flattening operation is useful for this phase of the method, but not so as regards the sifting by a current of air or other gas, the less so, as the space of the drum is filled with the whirled-up powder, and also the steel balls, 10 i. e. the continually falling balls, are therein contained. Therefore, it is preferable to effect the sifting in a separate space or chamber provided outside the drum, there being then used a stronger current by which not 15 only the finished foils are carried out, but also those which have only partly been finished at the time being and are conducted into the separator in which the first-mentioned foils and the other ones are separated 20 from one another, the latter being then returned to the drum in order to be treated again. In this way, also those finished foils which adhere to one another are removed 25 from the flattened drum. The use of a strong air or gas current is advantageous for the product.

While in the grinding of substances or materials of any kind in ball mills the attainment of as fine grains as possible is considered favorable, it is not so with the manufacture of bronze colors, in that there must in this case attention be paid to the particles retaining their shape as foils and that the area of the foils is not too small since otherwise the light-refracting capacity which gives to the bronze its particular and peculiar character ceases. Too small particles of bronze spoil the good appearance thereof and make it look "black", as experts term it. 40 Removing these particles later on by sifting is impossible, because their size or smallness is already below the meshes of the finest sieves having 10000 meshes per square centimeter. Besides, these too small particles have the 45 disagreeable characteristic that they commence to grind down the fine bronze foils whereby the final product is still more impaired. Finally, the absolutely necessary smooth and bright surface of the steel balls 50 is thereby destroyed.

With the known grinding procedure in a ball mill the mutual grinding down of the individual particles of the respective material is, as is known by experience, very important, if not decisive. But when operating in the manner in accordance with this invention, the ball mill behaves otherwise: it can then be caused to work the metal particles in such a manner that they are flattened and 60 form thin foils. Thus, the ordinary manner of operation of the ball mill is transformed into a procedure of quite another nature. If, however, this other manner of operation is ever and ever continued, it changes finally 65 automatically in such a way that the result-

ing product is a poorly-looking grey or brown powder. The difficulties are the greater, the finer the bronze is which is to be produced, and it is, therefore, of very great importance to prevent the flattening procedure from being transformed or converted into the ordinary manner of working of a ball mill. 70

Now, this is, according to the present invention, attained by the current of air or other gas passing through the mill being used in quite a distinct manner particularly suited to the purpose in view. While with the known procedure in the working of ball mills with the aid of a current of air stress is placed upon the production of as fine a powder as possible, and the air or gas current mentioned is used merely for carrying that powder out of the mill, without in any way affecting the shape of the grain, the air or gas current is employed, according to the present invention, to prevent such a fine powder from being produced and to remove the suitably thin foils flattened by the balls before they are converted into that fine 80 powder. In other words: the shape of the foils is affected by the said air or gas current. 85

Another object of the present invention is to increase the output by the carrying out of the flattening procedure in stages, i. e. in several phases or steps, in that the particles of the bronze are worked, in the first stage or stages, with tools capable of subjecting them to powerful blows; these tools may be larger 100 balls, or the ordinary balls may be dropped from a greater height. In this way, the particles are flattened preliminarily, and thereafter they are further treated with tools having a less pronounced effect. This can be done practically, for instance, in this way, that two flattening drums are used, the balls enclosed in the one drum being larger than the balls enclosed in the other drum, and the particles that have been treated in the 110 first drum being then conducted into the second drum and being therein treated until they are finished. 110

This manner of carrying out the method has the advantage (when a wind-operated sifter is provided outside the drums) to return those particles which are to be treated again exclusively to that drum in which the smaller balls are active or in which the height of fall of the balls is less. Returning said particles to the other drum would prove hurtful because in that case particles which have already been worked intensively would be worked in this manner a second time which would be too much. When, however, operating in the manner stated, the further advantage is attained that in the second drum continually a comparatively uniform powder mixture is contained. 120

Furthermore, by arranging the sifting or 125

separating device outside the drum or drums, a considerably shorter drum can be used, because in that case there does not exist the necessity of flattening all the particles completely within the drum so that they are finished when they leave the drum. Those not yet finished are returned from the sifter or separator to the drum.

The reduced length of the drum not only results saving of material, in connection with certain constructional advantages, but has, in addition thereto, the further advantage that the amount of the pulverulent material necessary to fill the drum so as to insure the desired effect can be correspondingly smaller. Cleaning the machine is now far simpler than heretofore.

The improved method can be carried out, for instance, with the aid of a machine as shown diagrammatically and by way of example on the accompanying drawings on which the main parts are shown in Figure 1 partly in vertical longitudinal section and partly in side-view; Figure 2 is a transverse section through the second drum (12) along line A—B in Fig. 1.

The material to be treated is contained in a receptacle 1 from which it is conveyed into the first flattening drum 4 through a pipe 3 by means of a conveying screw 2. In the drum 4 are enclosed steel balls 5, and at the ends of the drum are sieves 6 and 7 which let the bronze powder pass, but retain the steel balls. The bronze which has been treated in the drum by the balls leaves the drum through the sieve 7 and reaches a rotating chamber 8 provided with blades 9 of such a shape that the bronze powder is conveyed by them to an oblique chute 11 over which the powder passes into a vertical tube 10 through which the powder is introduced into the second drum 12. There are steel balls 15 in this drum, but they are smaller than the balls 5. Also the balls 15 are retained in the drum by sieves 13 and 14.

Both drums are supported on rolls upon which they can be, and are, rotated. I have abstained from showing also the means for this purpose, as they do not form part of the invention. It is obvious that any suitable means can be made use of for rotating said drums.

The current of air or gas which is to pass through the drum 12 is produced by means of a fan 16 which drives the respective fluid through a tube 17 into the tube 10. The current carries along in the drum the floating particles, that is to say, those which can pass through the meshes of the sieve 14. The mixture of the fluid and the particles of the bronze powder passes through the tube 18 into the upper chamber 19 of the sifting or separating device 20 which consists of an oblique casing in which are arranged superposed oblique plates 21 forming between them

passages 23 which communicate at their lower ends with an ante-chamber 24 communicating in turn with the upper chamber 19. The bronze powder falls down from this chamber upon the uppermost plate 21 and from the latter down into the chamber 24 or, more precisely, down upon the end of the next plate 21, and so on. The air or gas current entering the chamber 19 through the tube 18 and flowing from it into the chamber 24 is here subdivided into a plurality of smaller currents 23 flowing upwardly through between the plates 21, these currents carrying with it the finished particles, or the finished bronze powder respectively, which is now conveyed by said currents first into a collecting space 25 of the casing 20 and then further into a collecting vessel, a so-called cyclone separator, 26 from which finally it falls down into a conveying receptacle 27 of any suitable construction. The individual small air or gas currents pass through the pulverulent bronze while it drops from one of the plates 21 down to the next, and so on, until the remaining particles have arrived upon the oblique bottom of the casing 20. I wish it to be understood that instead of the cyclone separator 26 another, equivalent apparatus may be used for separating the bronze powder and the conveying fluid from one another.

The separating apparatus 26 is connected with the fan 16 by means of a tube 28. There is, thus, established a circuit composed of the members 16, 17, 10, 12, 18, 19, 24, 25, 26 and 28.

The particles which are not carried away by the said individual small air or gas currents, in that they are not yet in a finished state, pass through the branch 29 back into the drum 12 in order to be treated a second time.

As the circuit mentioned is completely closed it can be filled with an indifferent gas.

If desired, a filter or the like may be inserted between the apparatus 26 and the tube 28 in order to intercept also the finest, smallest, minute particles that may, perhaps, be carried away from said apparatus by the air or gas current flowing from it back to the fan 16.

The apparatus (cyclone separator or the like) 26 may be so designed that the bronze powder is subdivided in it according to the various sizes of the particles, and in that case there may be employed a corresponding number of collecting vessels 27.

Finally, instead of the separating device 20/21 any other, equivalent device may be used; or a sifting device with sieves may be used in connection with said device 20/21, or its equivalent.

I claim:

1. The method of producing metallic powders for use as bronze colors comprising

- flattening the metal particles by subjecting them to the action of smooth steel balls in a ball-mill, thereby converting the particles into small thin foils, continually supplying 5 fresh amounts of metal particles to said ball-mill at one end thereof and withdrawing the treated particles at the other end, passing a fluid current through said mill of such a strength as to carry off both finished and 10 unfinished particles, separating them outside said ball-mill and returning the unfinished particles thereto.
2. The method of producing metallic powders for use as bronze colors, comprising 15 flattening the metal particles in two stages by subjecting them in each stage to the action of steel balls in a ball-mill so as to produce flattened particles in the shape of small thin foils, the action of the steel balls in the first 20 stage being stronger than in the second stage, continually supplying fresh amounts of metal particles to be treated to the first ball-mill at one end thereof and withdrawing the treated particles at the other end, conveying said particles to the second ball-mill, passing a fluid current through said second ball-mill of such a strength as to carry off both finished and 25 unfinished particles, separating the same outside said last named ball-mill, and returning the unfinished particles to said ball-mill.
3. The method of producing metallic powders for use as bronze colors, comprising flattening the metal particles in two stages by subjecting them in each stage to the action 30 of smooth steel balls in a ball-mill so as to produce flattened particles in the shape of small thin foils, the flattening action in the first ball-mill being stronger than in the second ball-mill, continually supplying fresh metal 35 particles to the first ball-mill, withdrawing the treated particles from the second ball-mill by a fluid current of such a strength as to carry off both the finished and unfinished particles, separating them outside said second 40 ball-mill, and returning the unfinished particles to said second ball-mill.
- 45

In testimony whereof I affix my signature.  
ERWIN KRAMER.